



US006461526B1

(12) **United States Patent**  
**Wilson**

(10) **Patent No.:** **US 6,461,526 B1**  
(b4) **Date of Patent:** **\*Oct. 8, 2002**

(54) **METHOD FOR FORMING UNIFORM SHARP TIPS FOR USE IN A FIELD EMISSION ARRAY**

(75) Inventor: **Aaron R. Wilson**, Boise, ID (US)

(73) Assignee: **Micron Technology, Inc.**, Boise, ID (US)

(\*) Notice: Subject to any disclaimer, the term of this patent is extended or adjusted under 35 U.S.C. 154(b) by 68 days.

This patent is subject to a terminal disclaimer.

(21) Appl. No.: **09/639,357**

(22) Filed: **Aug. 14, 2000**

**Related U.S. Application Data**

(63) Continuation of application No. 09/026,243, filed on Feb. 19, 1998, now Pat. No. 6,171,164.

(51) **Int. Cl. 7** ..... **H01J 9/04**

(52) **U.S. Cl.** ..... **216/11; 216/24; 216/46; 216/51; 216/67; 216/79; 445/50**

(58) **Field of Search** ..... **445/24, 50, 51; 216/11, 24, 46, 51, 67, 79**

(56) **References Cited**

**U.S. PATENT DOCUMENTS**

4,983,878 A 1/1991 Lee et al.

|              |          |                             |
|--------------|----------|-----------------------------|
| 5,266,530 A  | 11/1993  | Bagley et al.               |
| 5,302,238 A  | 4/1994   | Roe et al.                  |
| 5,302,239 A  | 4/1994   | Roe et al.                  |
| 5,318,918 A  | 6/1994   | Frazier                     |
| 5,391,259 A  | * 2/1995 | Cathey et al. ..... 156/643 |
| 5,399,238 A  | 3/1995   | Kumar                       |
| 5,455,196 A  | 10/1995  | Frazier                     |
| 5,558,271 A  | 9/1996   | Rostoker et al.             |
| 5,561,328 A  | 10/1996  | Massingill et al.           |
| 5,627,427 A  | 5/1997   | Das et al.                  |
| 5,634,267 A  | 6/1997   | Farnsworth et al.           |
| 6,326,221 B1 | 12/2001  | Lee et al. ..... 438/20     |

\* cited by examiner

*Primary Examiner*—Anita Alanko

(74) *Attorney, Agent, or Firm*—TraskBritt

(57) **ABSTRACT**

A method of forming emitter tips for use in a field emission array is disclosed. The tips are formed by utilizing a polymer residue that forms during the dry etch sharpening step to hold the mask caps in place on the emitter tips. The residue polymer continues to support the mask caps as the tips are over-etched, enabling the tips to be etched past sharp without losing their shape and sharpness. The dry etch utilizes an etchant comprised of fluorine and chlorine gases. The mask caps and residue polymer are easily removed after etching by washing the wafers in a wash of deionized water, or Buffered Oxide Etch.

**38 Claims, 4 Drawing Sheets**





***Fig. 1***  
***(PRIOR ART)***



***Fig. 8***



Fig. 2



*Fig. 3*



*Fig. 4*



**Fig. 5**



**Fig. 6**



**Fig. 7**

**METHOD FOR FORMING UNIFORM SHARP  
TIPS FOR USE IN A FIELD EMISSION  
ARRAY**

**CROSS-REFERENCE TO RELATED  
APPLICATION**

This application is a continuation of application Ser. No. 09/026,243, filed Feb. 19, 1998, now U.S. Pat. No. 6,171,164 B1, issued Jan. 9, 2001.

**GOVERNMENT RIGHTS**

This invention was made with United States Government support under contract No. DABT63-97-C-0001 awarded by the Advanced Research Projects Agency (ARPA). The United States Government has certain rights in this invention.

**BACKGROUND OF THE INVENTION**

This invention relates generally to field emission displays and, more particularly, to the fabrication of an array of atomically sharp field tips for use in field emission displays.

The manufacture and use of field emission displays is well known in the art. The clarity, or resolution, of a field emission display is a function of a number of factors, including emitter tip sharpness.

One current approach toward the creation of an array of emitter tips is to use a mask to form the silicon tip structure, but not to form the tip completely. Prior to etching a sharp point, the mask is removed or stripped. Next, the tip is etched to sharpness after the mask is stripped from the apex of the tip.

It has been necessary to terminate the etch at or before the mask is fully undercut to prevent the mask from being dislodged from the apex. If an etch proceeds under such circumstances, the tips become lopsided and uneven due to the presence of the mask material along the side of the tip, or the substrate, during a dry etch and, additionally, the apex may be degraded, as shown in FIG. 1. Such a condition also leads to contamination problems because of the mask material randomly lying about a substrate. This mask 30, when dislodged, masks off a region of the substrate 11 where no masking is desired and allows continued etching in places where the mask 30 is supposedly protected. This results in randomly placed, undesired structures being etched in the material.

If the etch is continued after the mask is removed, the tip becomes more dull. This results because the etch chemicals remove material in all directions, thereby attacking the exposed apex of the tip while etching the sides. In addition, the apex of the tip may be degraded when the mask has been dislodged due to physical ion bombardment during a dry etch.

Accordingly, current methods perform underetching, which is to stop the etching process before a fine point is formed at the apex of the tip. Underetching creates a structure referred to as a "flat top." An oxidation step is then performed to sharpen the tip. This method results in a non-uniform etching across the array and the tips then have different heights and shapes. Other solutions have been to manufacture tips by etching, but they do not undercut the mask all the way. Furthermore, they do not continue etching beyond full undercut of the mask, as this typically leads to degradation of the tip. Rather, they remove the mask before the tip is completely undercut, then sharpen the tips from there. The wet silicon etch methods of the prior art result in

the mask being dislodged from the apex of the tip, at the point of full undercut. This approach can contaminate the bath, generate false masking, and degrade the apex.

The non-uniformity among the tips can also present difficulties in subsequent manufacturing steps used in the formation of the display. This is especially so in those processes employing chemical planarization, mechanical planarization or chemical mechanical planarization. Non-uniformity is particularly troublesome if it is abrupt, as opposed to a graduated change across the wafer.

Fabrication of the uniform wafer of tips using current processes is difficult to accomplish in a manufacturing environment for a number of reasons. For example, simple etch variability across the wafer affects the wafer at the time at which the etch should be terminated with the prior art approach.

Generally, it is difficult to obtain positive etches with definitions better than 5%, with uniformities of 10-20% being more common. This makes the "flat top" of an emitter tip etch using conventional methods vary in size. In addition, the oxidation necessary to "sharpen" or point the tip varies as much as 20%, thereby increasing the possibility of non-uniformity among the various tips in the array.

Tip height and other critical dimensions suffer from the same effects on uniformity. Variations in the masking 20 25 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630 9635 9640 9645 9650 9655 9660 9665 9670 9675 9680 9685 9690 9695 9700 9705 9710 9715 9720 9725 9730 9735 9740 9745 9750 9755 9760 9765 9770 9775 9780 9785 9790 9795 9800 9805 9810 9815 9820 9825 9830 9835 9840 9845 9850 9855 9860 9865 9870 9875 9880 9885 9890 9895 9900 9905 9910 9915 9920 9925 9930 9935 9940 9945 9950 9955 996

FIG. 2 is a cross-sectional schematic drawing of a pixel of a flat panel display having cathode emitter tips fabricated by the process of the present invention;

FIG. 3 is a cross-sectional schematic drawing of a substrate in which is deposited or grown a mask layer and a pattern photo resist layer, according to the process of the present invention;

FIG. 4 is a cross-sectional schematic drawing of the structure of FIG. 3, after the mask layer has been selectively removed by plasma dry etch, according to the process of the present invention;

FIG. 5 is a cross-sectional schematic drawing of the structure of FIG. 4, during the etch process of the present invention;

FIG. 6 is a cross-sectional schematic drawing of the structure of FIG. 5, as the etch proceeds according to the process of the present invention, illustrating that some of the tips become sharp before other tips;

FIG. 7 is a cross-sectional schematic drawing of the structure of FIG. 6, as the etch proceeds toward the process of the present invention; and

FIG. 8 is a cross-sectional schematic drawing of the structure of FIG. 7, depicting the sharp cathode tip after the etch has been completed and the mask layer has been removed.

#### DETAILED DESCRIPTION OF THE INVENTION

A representative portion of a field of emission display 10 is illustrated in FIG. 2. The emission display 10 includes a display segment 22. Each display segment 22 is capable of displaying a pixel, or a portion of a pixel 19, as, for example, one green dot of a red/green/blue full-color triad pixel. Preferably, a substrate comprised of glass is used and a material that is capable of conducting electric current is present on the surface of the substrate so that it can be patterned and etched to form micro cathodes or electrode emitter tips 13. Amorphous silicon is deposited on the glass substrate to form micro cathodes 13.

At a field emission site, a micro cathode 13 has been constructed on top of the substrate 11. The micro cathode 13 is a protuberance that may have a variety of shapes, such as pyramidal, conical, or other geometry that has a fine micro point for the emission of electrons. Surrounding micro cathodes 13 is a grid structure 15. When a voltage differential, through source 20, is applied between micro cathodes 13 and grid structure 15, a stream of electrons 17 is emitted toward a phosphor coated face plate 16. Face plate 16 serves as the anode where pixels 19 are charged by electrons 17.

The electron emission tip 13 is integral with a substrate 11 and serves as the cathode. Grid structure 15 serves as a grid structure for applying an electrical field potential to its respective micro cathode 13.

A dielectric insulating layer 14 is deposited on conductive micro cathode 13, which dielectric insulating layer 14 can be formed from the substrate or from one or more deposited films, such as a chromium amorphous silicon bilayer. Dielectric insulating layer 14 also has an opening at the field emission site location.

Disposed between face plate 16 and base plate 21 are spatial support structures 18 that function as support for atmospheric pressure that exists on the electrode face plate 16. The atmospheric pressure is the result of the vacuum created between the base plate 21 and face plate 16 for the proper functioning of the emitter tips 13.

Base plate 21 comprises a matrix addressable array of cold cathode emitter tips 13, a substrate 11 where tips 13 are formed, dielectric insulating layer 14, and anode grid structure 15.

In the process of the present invention, the mask dimensions, the balancing of the gases and parameters in the plasma etch enable the manufacturer to determine and significantly control the dimensions of tip 13. Compositions of the mask affects the ability of mask 30 to remain balanced at the apex of the emitter tip 13 and to remain centered on the apex of emitter tip 13 during the over-etching of tip 13. This is achieved by using a combination of gases that forms a polymer support between the apex of tip 13 and the subsurface of dielectric insulating layer 14, rather than merely relying upon mask 30 to balance precariously on the emitter tip 13 during the etching process. Over-etching refers to the time period when the etch process is continued after a substantially full undercut is achieved. Full undercut refers to the point at which the lateral removal of material is equal to the original lateral dimension of the mask 30.

FIG. 3 depicts the substrate 11, which is amorphous silicon overlying glass, polysilicon, or any other material from which emitter tip 13 can be fabricated. Substrate 11 has a mask layer 30 deposited or grown thereon. Mask layer 30 is typically a 0.2 micrometer ( $\mu\text{m}$ ) layer of silicon dioxide formed on the substrate 11. Tip geometries and dimensions and conditions for the etch process will vary with the type of materials used to form tips 13.

Mask layer 30 can be made of any suitable materials such that its thickness is great enough to avoid being completely consumed during the etching process, but not so thick as to overcome the adherent forces that maintain it in the correct position with respect to tip 13 throughout the etch process.

A photo resist layer 32, or other protective element, is patterned on mask layer 30 if the desired masking material cannot be directly patterned or applied. When photo resist layer 32 is patterned, the preferred shapes are dots or circles.

The next step in the process is selective removal of mask 30 that is not covered by photo resist pattern 32 as shown in FIG. 4. The selective removal of mask 30 is accomplished preferably through a wet chemical etch. An aqueous HF solution can be used in a case of a silicon dioxide mask; however, any suitable technique known in the industry may also be employed, including physical removal techniques or plasma removal.

In a plasma etch, the typical etches used to etch the silicon dioxide include, but are not limited to: Chlorine and Fluorine. And typical gases and compounds include:  $\text{CF}_4$ ,  $\text{CHF}_3$ ,  $\text{C}_2\text{F}_6$  and  $\text{C}_3\text{F}_8$ . Fluorine with oxygen can also be used to accomplish the oxide mask 30 etch step. The etchant gases are selective with respect to silicon and the etch rate of oxide is known in the art, so that the point of the etch step can be calculated.

Alternatively, a wet oxide etch can also be preformed using common oxide etch chemicals. At this stage, the photo resist layer 32 is stripped. FIG. 5 depicts the mask 30 structure prior to the silicon etch step.

A plasma etch, with selectivity to the etch mask 30, is then employed to form tips 13. The plasma contains a fluorinated gas, such as  $\text{NF}_3$ , in combination with a chlorinated gas, such as  $\text{Cl}_2$ , and forms a polymer residue that supports the mask during the etch process. Preferably, the plasma comprises a combination of  $\text{NF}_3$  and  $\text{Cl}_2$ , and an additive, such as helium. The combination of  $\text{NF}_3$  and  $\text{Cl}_2$  is in such a ratio that during the etching process, a polymer 34 is formed underneath mask 30 and on the tip 13. Polymer 34 is used

to build a mask support of mask 30 as tip 13 goes from before sharp, shown in FIG. 5, to etch sharp, shown in FIG. 6, and past sharp, shown in FIG. 7. Sharpness is defined as “atomically sharp” and refers to a degree of sharpness that cannot be defined clearly by the human eye when looking at a scanning electron microscope (SEM) micrograph of the structure. The human eye cannot distinguish where the peak of tip 13 actually ends. The measured apex of a sharp tip is typically between 7 Å and 10 Å.

The following are the ranges of parameters for the process as described in the present application. Included is a range of values investigated during the characterization of the process, as well as the range of values that provides the best results for tips 13 that were from 1  $\mu\text{m}$  to 2  $\mu\text{m}$  in height and 1.3  $\mu\text{m}$  to 2.0  $\mu\text{m}$  at the base, with 1.5  $\mu\text{m}$  preferred. One having ordinary skill in the art will realize that the values can be varied to obtain a tip 13 having other height and width dimensions previously stated.

TABLE 1

| Parameters                             | Investigative Range | Preferred Range |
|----------------------------------------|---------------------|-----------------|
| Cl <sub>2</sub> :NF <sub>3</sub> ratio | 10 to 60%           | 30 to 40%       |
| Cl <sub>2</sub> :NF <sub>3</sub>       | 150–620 SCCM        | 290–340 SCCM    |
| Helium                                 | 60–250 SCCM*        | 110–140 SCCM    |
| Power                                  | 2500 w              | 2500 w          |
| Pressure                               | 5–100 mTorr         | 50–70 mTorr     |
| Bottom Electrode Power                 | 0–400 w             | 200–300 w       |
| Spacing Time                           | 1.5–3.5 min         | 140–150 seconds |
| Temperature                            | 15–70° C.           | 35–45° C.       |

\*SCCM - Standard Cubic Centimeters per Minute

Experiments were conducted on a LAM continuum etcher with enhanced cooling. The lower electrode was maintained substantially in the range of 40° C. The etched time that received the best results was between 140–150 seconds with 145 seconds being optimal.

The use of the polymer 34 created during the etching allows the tips to achieve an aspect ratio of 2.5–3.2 using the preferred parameter ranges. Aspect ratio=downward etch rate/undercut etch rate.

The ability to etch to its conclusion past full undercut with minimal changes to the functional shape between the first tip 13 to become sharp and the last tip to become sharp provides a process in which all of the tips in the array are essentially identical in characteristics. Tips of uniform height and sharpness are carefully selected based on the ratio of NF<sub>3</sub> to Cl<sub>2</sub> used during the mask etch step. This is important in that the combination of NF<sub>3</sub> to Cl<sub>2</sub> forms the polymer 34 that provides support for mask 30 during the etching of emitter tips 13.

After the array of emitter tips 13 has been fabricated, the oxide mask layer 30 can be removed along with the polymer layer 34. This is illustrated in FIG. 8. Mask layer 30 and polymer 34 are stripped off by a simple wet etch utilizing deionized water, or a Buffered Oxide Etch. As the mask layer has been etched away from each tip 13, no harsh chemicals need to be used during a subsequent etch removal of mask layer 30.

Ideally, the NF<sub>3</sub>—Cl<sub>2</sub> gas is provided at 310 SCCMs while the helium gas is provided at 125 SCCMs during etching.

The yield of tips results in a uniformity of 20%, or within plus or minus 10%, of the average height and shape for each tip 13. Further, the yield is improved such that a fewer number of tips per pixel are necessary as more and more useful tips are provided. Additionally, with the more-

uniform height and sharpness, the turn-on voltage during operation of a field emission display can be lowered. Further, the number of shorter tips that are much shorter than the dimension desired are greatly reduced or eliminated, which means shorting to the grid is also reduced or eliminated.

While the particular process for forming sharp emitter tips to use in flat panel displays as herein shown and disclosed in detail is fully capable of obtaining the desired effects stated above, it is to be understood that it is to be illustrated as the presently preferred embodiments of the invention and that no limitations are intended to the details of construction or design herein shown other than as described in the depending claims. For example, the process of the present invention was discussed with regards to the fabrication of uniform arrays of sharp emitter tips and flat panel displays; however, one of ordinary skill in the art will realize that such a process can be applied to other field ionizing and electron emitting structures, and to micro-machining of structures in which it is desired to have a sharp point, such as a probe tip or other device.

What is claimed is:

1. A method of forming a substantially uniform array of emitter tips comprising:  
providing a mask;  
masking a substrate using the mask;  
etching said substrate to form an array of pointed tips;  
forming a polymer support on said pointed tips to support said mask; and  
removing said mask and said polymer support.
2. The method according to claim 1, wherein said mask is a hard mask.
3. The method according to claim 1, wherein said mask is patterned as an array of circles.
- 35 4. The method according to claim 3, wherein said circles have diameters of approximately 1.5  $\mu\text{m}$ .
5. The method according to claim 1, wherein said etching step includes etching said array of pointed tips until substantially a majority of said tips of said array of pointed tips are sharp.
- 40 6. The method according to claim 1, wherein said etching step utilizes a dry etchant comprised of a fluorine gas and a chlorine gas.
7. The method according to claim 6, wherein said fluorine gas is comprised of NF<sub>3</sub>.
- 45 8. The method according to claim 6, wherein said chlorine gas is comprised of Cl<sub>2</sub>.
9. The method according to claim 6, wherein said chlorine gas and said fluorine gas are provided in a range of about 10% to about 60% chlorine.
- 50 10. The method according to claim 6, wherein said chlorine gas ranges from 30%–40% to said fluorine and a chlorine gas.
11. The method according to claim 6, wherein said dry etchant further includes an inert gas.
- 55 12. The method according to claim 6, wherein said dry etchant is provided in a range from about 150 SCCM to about 620 SCCM.
13. The method according to claim 6, wherein said dry etchant is provided in a range from about 290 SCCM to about 340 SCCM.
- 60 14. The method according to claim 11, wherein said inert gas is provided in a range from about 60 SCCM to about 250 SCCM.
- 65 15. The method according to claim 1, wherein said etching step is performed for a period of time in the range of about 1.5 minutes to about 3.5 minutes.

16. The method according to claim 1, wherein said etching step is performed for a period of time in the range of about 140 seconds to about 150 seconds.

17. The method according to claim 1, wherein said etching step is performed at a temperature in the range of about 15° C. to about 70° C.

18. The method according to claim 1, wherein said etching step is performed in a temperature range from about 35° C. to about 45° C.

19. The method according to claim 1, wherein said etching step is performed for a period of time of about 145 seconds at a temperature of about 40° C.

20. A method of forming a substantially uniform array of emitter tips comprising:

providing a mask having an array including a plurality of 15 circles;

masking a substrate to define a mask array;

etching said substrate to form an array of pointed tips; forming a polymer support on said pointed tips to support 20 a mask; and

removing said mask and said polymer support.

21. The method according to claim 20, wherein said mask is a hard mask.

22. The method according to claim 20, wherein said mask includes a mask patterned as an array of one of a plurality of circles and a plurality of dots.

23. The method according to claim 22, wherein said circles have a diameter of approximate range of 1.5  $\mu\text{m}$ .

24. The method according to claim 20, wherein said etching includes etching said array of pointed tips until a substantially majority of said tips of said array of pointed tips are sharp.

25. The method according to claim 20, wherein said etching step utilizes a dry etchant comprised of a fluorine gas and a chlorine gas.

26. The method according to claim 25, wherein said fluorine gas is comprised of  $\text{NF}_3$ .

27. The method according to claim 25, wherein said chlorine gas is comprised of  $\text{Cl}_2$ .

28. The method according to claim 25, wherein said chlorine gas and said fluorine gas are provided in a range of about 10% to about 60% chlorine.

29. The method according to claim 25, wherein said chlorine gas ranges from about 30% to about 40% to said fluorine and chlorine gases.

30. The method according to claim 25, wherein said dry etchant further comprises an inert gas.

31. The method according to claim 25, wherein said dry etchant is provided at a rate in the range of about 150 SCCM to about 620 SCCM.

32. The method according to claim 25, wherein said dry etchant is provided in a range from about 290 SCCM to about 340 SCCM.

33. The method according to claim 30, wherein said inert gas is provided in a range from about 60 SCCM to about 250 SCCM.

34. The method according to claim 20, wherein said etching step is performed for period of time in the range from about 1.5 minutes to about 3.5 minutes.

35. The method according to claim 20, wherein said etching step is performed for a period of time in the range from about 140 seconds to about 150 seconds.

36. The method according to claim 20, wherein said etching step is performed in a temperature range from about 15° C. to about 70° C.

37. The method according to claim 20, wherein said etching step is performed in a temperature range from about 35° C. to about 45° C.

38. The method according to claim 20, wherein said etching step is performed for a period of time of about 145 seconds at a temperature of about 40° C.

\* \* \* \* \*

UNITED STATES PATENT AND TRADEMARK OFFICE  
**CERTIFICATE OF CORRECTION**

PATENT NO. : 6,461,526 B1  
DATED : October 8, 2002  
INVENTOR(S) : Aaron R. Wilson

Page 1 of 1

It is certified that error appears in the above-identified patent and that said Letters Patent is hereby corrected as shown below:

Column 3.

Line 51, change "emission" to -- emitter --

Column 4.

Line 24, after "a" and before "mask" insert -- mask or --

Line 39, change "pattern" to -- layer --

Column 6.

Line 18, change "election" to -- electrode --

Line 66, before "range" change "the" to -- a --

Column 7.

Line 2, before "range" change "the" to -- a --

Line 5, before "range" change "the" to -- a --

Column 8.

Line 12, before "range" change "the" to -- a --

Line 21, before "range" change "the" to -- a --

Line 34, before "range" change "the" to -- a --

Signed and Sealed this

Sixteenth Day of September, 2003



JAMES E. ROGAN  
*Director of the United States Patent and Trademark Office*